

# United States Patent [19]

Blackburn et al.

[11] Patent Number: 4,820,356

[45] Date of Patent: Apr. 11, 1989

[54] HEAT TREATMENT FOR IMPROVING FATIGUE PROPERTIES OF SUPERALLOY ARTICLES

[75] Inventors: Martin J. Blackburn, Kensington; Daniel F. Paulonis, Higganum; Robert H. Caless, Bolton; Anne L. D'Orvilliers, Hartford, all of Conn.

[73] Assignee: United Technologies Corporation, Hartford, Conn.

[21] Appl. No.: 137,853

[22] Filed: Dec. 24, 1987

[51] Int. Cl.<sup>4</sup> ..... C22F 1/10

[52] U.S. Cl. ..... 148/12.7 N; 148/162; 148/410

[58] Field of Search ..... 148/162, 12.7 N, 410, 148/409

[56]

## References Cited

### U.S. PATENT DOCUMENTS

4,608,094 8/1986 Miller et al. ..... 148/410

Primary Examiner—R. Dean  
Attorney, Agent, or Firm—Charles E. Sohl

## [57] ABSTRACT

Heat treatments are described for improving the fatigue properties of superalloy articles, without adversely affecting other mechanical properties. The entire heat treatment process is performed below the gamma prime solvus temperature so that significant grain growth does not occur. The heat treatment cycle causes the formation of gamma prime particles in a controlled manner and morphology, first at the grain boundaries and then within the grains. The resultant microstructure possesses the benefits of a fine grain structure (improved resistance to fatigue crack initiation) and fine gamma prime particle size (improved resistance to crack growth).

8 Claims, 5 Drawing Sheets



H.T. = Heat Treatment  
G.P.S. = Gamma Prime Solvus

F/G.1

H.T. = Heat Treatment  
G.P.S. = Gamma Prime Solvus



FIG. 2



FIG. 3

F/FIG. 4

T=1100°F

f= 10 cpm



F/G. 5 $T=1100\text{ F}$  $f=10\text{ cpm}$ 

# HEAT TREATMENT FOR IMPROVING FATIGUE PROPERTIES OF SUPERALLOY ARTICLES

## TECHNICAL FIELD

The invention relates to heat treatments for superalloy articles to improve fatigue properties.

## BACKGROUND ART

Superalloys are materials, usually nickel based, which have useful properties at temperatures on the order of 1000° F. and above and which are widely used in gas turbine engines. Nickel base superalloys generally consist of a gamma (nickel solid solution) matrix containing a strengthening array of gamma prime phase ( $Ni_3Al$  type) particles. The particle size and distribution can be altered by heat treatment and this also alters the mechanical properties of the alloy.

One important gas turbine engine application for superalloys is turbine and compressor disks. Disks are internal engine components which support and locate the blades in the gas path. In engine operation the disk rotates at speeds of up to about 10,000 rpm (and higher in small engines) and experience temperatures ranging from up to about 1500° F. at the rim to about 500° F. at the center, known as the bore. Disks must have high tensile strength and high creep and stress rupture resistance. In addition, the disk experiences cyclic stresses which can lead to failure if the fatigue properties are inadequate.

While the invention development focused on disk applications, the invention is not so limited.

These property requirements, in the context of the high temperature environment, have led to the use of superalloy disks in virtually all modern turbine engines. Despite the generally acceptable properties exhibited by currently used disks, there is still a need for components which have yet better properties. Improved disk properties can translate into longer disk lives, lighter engines, or permit engine operation at higher rotational speeds.

As noted above, the properties of superalloys can be altered by heat treatment. Many prior art heat treatment developments for disk materials have included heating above the gamma prime solvus temperature. When the gamma prime solvus temperature is exceeded all the gamma prime dissolves leaving nothing to retard grain boundary motion. This leads to rapid grain growth and results in a coarse grain structure, which usually reduces tensile strength and fatigue initiation life but often improves (reduces) the crack growth rate. Conversely, conventional fine grain structures display long times to fatigue crack initiation but then exhibit relatively rapid crack growth rates.

The invention is a heat treatment which provides a fine grain structure that is more resistant to crack initiation and has a lower crack growth rate than prior art treated fine grain material.

Typical of the art are U.S. Pat. Nos. 4,608,094 and 4,624,716. Pending, commonly assigned, U.S. Application No. 733,446 filed 5/10/85 describes a heat treatment for reducing the fatigue susceptibility of gas turbine engine disks, this pending application is currently the subject of a U.S. Patent Office Secrecy Order.

## DISCLOSURE OF INVENTION

The present invention is a heat treatment process which will often be applied to forgings especially those

produced according to U.S. Pat. No. 3,519,503, although it also has application to disks produced by other means such as HIP (hot isostatic pressed) powder and disks conventionally forged from ingot starting material. The invention is applicable to nickel base superalloys containing from about 40 to about 70 volume percent of the gamma prime phase. Table I lists several exemplary superalloys and a general disk alloy composition range which can be processed according to the invention.

The starting articles will have a grain size which has been established by the prior thermal mechanical history of the part. In the case of forgings, the grain size will be relatively fine as a result of recrystallization which generally occurs during forging. A typical grain size for disk forgings is ASTM 8 to 12, (0.022-0.006 mm average grain diameter respectively).

An important characteristic of the invention process is that this starting grain size is held essentially constant throughout the process. Preferably the starting grain size does not change by more than about one ASTM unit during the invention process.

FIG. 1 is a block diagram which illustrates the invention steps. FIG. 2 is a schematic diagram of the invention process. Tables II, III and IV illustrate suggested parameters for several widely used disk materials as employed in small, moderate and large parts and the notation in Tables II, III and IV follows that in FIG. 2.

The first step (I) in the process develops coarse grain boundary gamma prime by a subsolvus solution treatment which puts the majority of the gamma prime into solid solution but retains a sufficient amount (at least about 10 volume %) as precipitates to prevent significant grain growth. This heat treatment will be performed at a first heat treat temperature which is 5°-50° F. below the gamma prime solvus and preferably 15°-40° F. below the gamma prime solvus for at least 0.5 hour and preferably 1-10 hours. After this step the part will have some gamma prime retained out of solution (as precipitates) but most of the gamma prime will be in solution. From this first heat treat temperature the articles are cooled at a controlled rate of from about 20°-200° F. per hour and preferably 50°-150° F. per hour to a temperature which is at least 200° F. below the first heat treatment temperature and preferably at least 300° F. below the first heat treatment temperature. This controlled cooling step causes controlled preferential precipitation and growth of coarse gamma prime particles at the grain boundaries, the particles being approximately 1-5 microns in diameter. After the controlled cooling step, the article can be rapidly cooled to room temperature.

The second step (II) in the invention process develops a distribution of fine gamma prime precipitates within the grains and comprises heating the part to a second heat treatment temperature about 10°-250° F. below the first heat treat temperature for a time of at least 0.5 hours and preferably 1-10 hours. This heat treatment again dissolves or solutionizes a portion of the gamma prime particles but grain growth is again prevented. After this step the article is rapidly cooled to room temperature (actually, only the cooling rate down to about 1200° F. affects the gamma prime size, below about 1200° F. the cooling rate is unimportant). In this context rapid cooling means at least as fast as forced air cooling (typically 600° F. in 15 minutes for a 4 inches thick 300 lb. disk) and possibly faster depending on part

size. The cooling rate must be sufficiently fast that, after a subsequent tempering step described below, the intra-granular gamma prime size is within a critical size range.

This cooling rate in combination with alloy composition, heat treatment temperature and part size and geometry determines the gamma prime particle size within the grains. These relations are complex and require experimental optimization for each combination of alloy and part geometry to achieve a fine internal gamma prime particle size.

Small parts achieve an actual cooling which is close to the gross cooling rate imposed on the part. However, for large parts the thermal mass does not permit achievement of rapid actual cooling rates throughout the part so the actual internal cooling can be relatively slow.

Parts of sizes which are compatible with a rapid actual cooling rate can be heat treated very near, but below the gamma prime solvus, and achieve the desired fine gamma prime particle size. However, parts which experience a slow actual cooling rate must be quenched from lower temperatures, i.e. 100°-300° F. below the gamma prime solvus, to achieve the gamma prime particle size within the desired range.

The inventors have noted a relationship between average precipitate (non grain boundary) gamma prime size and crack growth resistance. This is illustrated in FIG. 3 with maximum crack growth resistance being observed for particle sizes having an average size of less than about 0.15 micron (and preferably less than 0.1 micron). It is not known if there is an actual lower limit but about 0.02 micron is a practical lower limit since the high cooling rates needed to obtain finer sizes are presently impractical.

As previously suggested, it is necessary to vary the second subsolution treatment temperature and cooling rate for a particular part geometry to achieve the desired gamma prime precipitate particle size. Specifically, small parts treated according to this invention (small parts being defined as having a thickness of less than about 1.0 inch and/or weight of less than about 20 pounds) can be forced air cooled (or of course cooled even faster) from a relatively high subsolution treatment temperature, whereas large parts (parts more than about 2 inches thick and/or weighing more than about 100 pounds) must be liquid quenched from a lower subsolution treatment temperature to achieve a comparable fine gamma prime size. For intermediate size parts, (weighing between about 20 and about 100 pounds and/or having a thickness from about 1 to 2 inches, it has been found satisfactory to use a lower subsolution treatment temperature in combination with forced air cooling. This gives a comparable fine gamma prime particle size. Many actual components will have sections or different thicknesses. In such cases, heat treatment parameter compromise is necessary, preferably biased in favor of those sections having the greatest need for fatigue resistance.

The third step in the process is an aging or stabilization step accomplished by heating the article to a third heat treatment temperature of about 1200°-1500° F. for 1-25 hours. This equilibrates the gamma prime particles. Multistep stabilization steps may also be used.

At the conclusion of the invention heat treatment process the article will have a fine grain size which approximates that of the starting grain size with concentration of coarse (1-5 microns average diameter)

gamma prime particles at the grain boundaries and a very fine (0.02-0.15 average diameter) uniform gamma prime dispersion within the grains. This structure has been found to provide greatly enhanced crack growth resistance as compared to the prior art microstructures. In addition, since the fine starting grain size is retained, the inherent resistance of a fine grain structure to crack initiation is also retained.

Large size parts will quite likely contain significant internal stresses resulting from the rapid (liquid) cooling step. These stresses can be detrimental in subsequent processing and in eventual service. Residual stresses can be ameliorated by stressing the part sufficiently to cause localized yielding thereby relieving some of the internal stress. For gas turbine engine disks, this stressing can be achieved by spinning the disk and thereby developing centrifugal stresses sufficient to cause slight local yielding. Other stress relief methods may also be employed.

The preceding description of the process outlined in FIG. 1 is the preferred process and is a process which will give the optimum results. FIG. 1 shows a dotted line which bypasses the initial subsolvus treatment and the controlled cooling rate. If this dotted line is followed, the starting material having initial grain size of ASTM 8-12, and the characteristic gamma prime solvus temperature will be processed according to the lower portion of the Figure depending on its size as a small, medium or large part. This processing sequence will produce an improvement in crack growth rate about half that which would be produced by the entire process.

FIG. 4 shows the effect of the invention process on the fatigue life of MERL 76 alloy. The "prior art" curve shows crack growth behavior for conventionally processed MERL 76 material. The "preferred invention" curve shows behavior of MERL 76 material given the complete invention process. The intermediate curve, "modified invention", is for material given a treatment wherein the first heat treatment was eliminated. It can be seen that elimination of the first heat treatment reduces the invention benefit by about half.

The foregoing, and other features and advantage of the present invention will become more apparent from the following description of preferred embodiments and accompanying drawings.

#### BRIEF DESCRIPTION OF DRAWINGS

FIG. 1 is a block diagram of the invention process.

FIG. 2 is a schematic diagram of the invention process.

FIG. 3 shows the fatigue life resulting from different gamma prime particle sizes.

FIG. 4 shows the effect of two versions of the invention process on the fatigue behavior of MERL 76.

FIG. 5 shows the fatigue life benefit for large parts resulting from the invention process (with and without the stressing step).

#### BEST MODE FOR CARRYING OUT THE INVENTION

The invention process has been previously described and is illustrated schematically in FIGS. 1 and 2. The information in Tables I-IV in combination with that description will enable one skilled in the art to practice the invention process on a variety of commonly used superalloy disk materials. What follows are several illustrative examples.

## EXAMPLE 1

This example describes the processing of small, 20 pound, MERL 76 (whose gamma prime solvus is about 2175° F.) parts for optimum fatigue resistance. The correct coarse gamma prime grain distribution, concentrated mainly at grain boundaries is established using a first heat treatment at 2140° F. for 2 hours followed by forced air cooling at a rate of approximately 100° F. per hour to 1800° F. and then cooling to room temperature.

The next step produces a very fine gamma prime dispersion within the grains, by heat treating at 2075° F. for 2 hours and then forced air cooling to room temperature. The parts are then aged at 1350° F. for 16 hours.

## EXAMPLE 2

Another small MERL 76 part was processed as described in Example 1 except that the first heat treatment step (at 2140° F.) and subsequent controlled cooling was omitted.

## EXAMPLE 3

This example illustrates a prior art treatment applied to small MERL 76 components.

Solution: 2090° F./2 hours/oil quench

Stabilize: 1800° F./1 hour/forced aircool

Age: 1350° F./8 hours/air cool

FIG. 4 illustrates the crack growth (da/dN) behavior of the material processed according to example 1, the invention process, Example 2, the shortened or modified invention process and Example 3, the prior art process. It can be seen that the invention process provides a substantial improvement in crack growth behavior and that the shortened invention step produces a reduced benefit.

## EXAMPLE 4

This example deals again with the MERL 76 material but teaches how to heat treat this material in large size components, namely components having a thickness of greater than about 2 inches and/or weighing more than about 100 pounds. Typical of such articles would be gas turbine disk forgings. Such thick starting sections are subsolution treated at 2140° F. for 2 hours and then furnace cooled at about 100° F. per hour to 1900° F. and then forced air cooled to room temperature. The forgings are then heat treated at 1975° F. for 2 hours and oil quenched. The final step is a 1350° F. stabilization treatment for sixteen hours.

## EXAMPLE 5

This example illustrates an optional but highly advantageous invention step applicable to large size parts which have been liquid quenched. Such parts contain substantial residual stresses as a result of cooling in a liquid media. Such varying residual stresses produce highly variable fatigue results. In Example 5 a large part of the same geometry and same material as that in Example 4 was given all the heat treatment steps described in Example 4 but was then proof stressed by spinning the material at room temperature at a speed which developed stresses sufficient to overcome the quench caused stresses. The quenched part contained complex internal stresses, compressive at the surface balanced by internal tensile stresses. Such stresses vary in magnitude and sense within the part. The object of the post quench stress step is to impose external stresses sufficient to cause some local internal yielding, thereby reducing

some of the quench developed residual stresses. Substantial scatter in fatigue properties was noted for samples taken from the non-spun disk compared with samples taken from the stressed disk. This is shown in FIG. 5 where the cross hatched area comprises the reduction in scatter. The line denoted "Goal" is the crack growth typical of Waspaloy, a crack growth resistant prior art material which is substantially inferior in strength to the alloys described in Table I and a clear reduction in the scatter band can be seen. This undesirable scatter was markedly reduced in the disk which was stressed by spinning. This scatter reduction is very desirable and the stress step is a preferred invention step.

Table V shows other typical mechanical properties of invention (the process including the first heat treat step) processed material and prior art processed material (both IN100 material). It can be seen that the invention process slightly reduces the yield strength but does not affect other properties.

Although this invention has been shown and described with respect to detailed embodiments thereof, it will be understood by those skilled in the art that various changes in form and detail thereof may be made without departing from the spirit and scope of the claimed invention.

TABLE I

|      | Nominal Composition, Wt % |          |           |          | Broad Range Disk Alloys |
|------|---------------------------|----------|-----------|----------|-------------------------|
|      | MERL 76                   | IN100    | Astro-loy | Rene 95  |                         |
| Cr   | 12.4                      | 12.35    | 15.0      | 14.0     | 10-20                   |
| Co   | 18.5                      | 18.50    | 17.0      | 8.0      | 5-20                    |
| Mo   | 3.2                       | 3.20     | 5.0       | 3.5      | 0-6                     |
| W    | —                         | —        | —         | 3.5      | 0-6                     |
| Ta   | —                         | —        | —         | 3.5      | 0-5                     |
| Cb   | 1.4                       | —        | —         | —        | 0-4                     |
| Al   | 5.0                       | 4.95     | 4.0       | 3.5      | 2-6                     |
| Ti   | 4.3                       | 4.35     | 3.5       | 2.5      | 1-5                     |
| V    | —                         | 0.78     | —         | —        | 0-1                     |
| C    | 0.025                     | 0.07     | 0.06      | 0.15     | 0.01-0.2                |
| B    | 0.02                      | 0.02     | 0.03      | 0.010    | 0.01-0.05               |
| Zr   | 0.06                      | 0.06     | —         | 0.05     | 0.02-0.08               |
| Hf   | 0.40                      | —        | —         | —        | 0-1.0                   |
| Ni   | Balance                   | Balance  | Balance   | Balance  | Balance                 |
| GPST | 2175° F.                  | 2140° F. | 2075° F.  | 2100° F. | (Varies)                |

(GPST = Gamma Prime Solvus Temp.)

TABLE II

|                          | Typical Small Part Invention Process Parameters |             |             |             |
|--------------------------|-------------------------------------------------|-------------|-------------|-------------|
|                          | MERL 76                                         | IN100       | ASTRO-LOY   | RENE 95     |
| Gamma Prime Solvus Temp. | 2175° F.                                        | 2140° F.    | 2075° F.    | 2100° F.    |
| <u>I</u>                 |                                                 |             |             |             |
| a. temp.                 | 2140° F.                                        | 2105° F.    | 2040° F.    | 2065° F.    |
| b. time                  | 2 hrs.                                          | 2 hrs.      | 2 hrs.      | 2 hrs.      |
| c. cooling rate          | 100° F./hr.                                     | 100° F./hr. | 100° F./hr. | 100° F./hr. |
| d. controlled cool end   | 1900° F.                                        | 1850° F.    | 1800° F.    | 1800° F.    |
| <u>II</u>                |                                                 |             |             |             |
| a. temp.                 | 1975° F.                                        | 1940° F.    | 1875° F.    | 1900° F.    |
| b. time                  | 2 hrs.                                          | 2 hrs.      | 2 hrs.      | 2 hrs.      |
| c. cooling technique     | forced air                                      | forced air  | forced air  | forced air  |
| <u>III</u>               |                                                 |             |             |             |
| a. temp.                 | 1350° F.                                        | 1350° F.    | 1350° F.    | 1350° F.    |
| b. time                  | 16 hrs.                                         | 16 hrs.     | 16 hrs.     | 16 hrs.     |

TABLE III

| Typical Medium Part Invention Process Parameters |             |             |               |             |
|--------------------------------------------------|-------------|-------------|---------------|-------------|
|                                                  | MERL<br>76  | IN100       | ASTRO-<br>LOY | RENE<br>95  |
| Gamma Prime Solvus Temp.                         | 2175° F.    | 2140° F.    | 2075° F.      | 2100° F.    |
| <u>I</u>                                         |             |             |               |             |
| a. temp.                                         | 2140° F.    | 2105° F.    | 2040° F.      | 2065° F.    |
| b. time                                          | 2 hrs.      | 2 hrs.      | 2 hrs.        | 2 hrs.      |
| c. cooling rate                                  | 100° F./hr. | 100° F./hr. | 100° F./hr.   | 100° F./hr. |
| d. controlled cool end                           | 1900° F.    | 1850° F.    | 1800° F.      | 1800° F.    |
| <u>II</u>                                        |             |             |               |             |
| a. temp.                                         | 1975° F.    | 1940° F.    | 1895° F.      | 1900° F.    |
| b. time                                          | 2 hrs.      | 2 hrs.      | 2 hrs.        | 2 hrs.      |
| c. cooling technique                             | forced air  | forced air  | forced air    | forced air  |
| <u>III</u>                                       |             |             |               |             |
| a. temp.                                         | 1350° F.    | 1350° F.    | 1350° F.      | 1350° F.    |
| b. time                                          | 16 hrs.     | 16 hrs.     | 16 hrs.       | 16 hrs.     |

TABLE IV

| Typical Large Part Invention Process Parameters |             |             |               |             |
|-------------------------------------------------|-------------|-------------|---------------|-------------|
|                                                 | MERL<br>76  | IN100       | ASTRO-<br>LOY | RENE<br>95  |
| Gamma Prime Solvus Temp.                        | 2175° F.    | 2140° F.    | 2075° F.      | 2100° F.    |
| <u>I</u>                                        |             |             |               |             |
| a. temp.                                        | 2140° F.    | 2105° F.    | 2040° F.      | 2065° F.    |
| b. time                                         | 2 hrs.      | 2 hrs.      | 2 hrs.        | 2 hrs.      |
| c. cooling rate                                 | 100° F./hr. | 100° F./hr. | 100° F./hr.   | 100° F./hr. |
| d. controlled cool end                          | 1900° F.    | 1850° F.    | 1800° F.      | 1800° F.    |
| <u>II</u>                                       |             |             |               |             |
| a. temp.                                        | 1975° F.    | 1940° F.    | 1875° F.      | 1900° F.    |
| b. time                                         | 2 hrs.      | 2 hrs.      | 2 hrs.        | 2 hrs.      |
| c. cooling technique                            | oil quench  | oil quench  | oil quench    | oil quench  |
| <u>III</u>                                      |             |             |               |             |
| a. temp.                                        | 1350° F.    | 1350° F.    | 1350° F.      | 1350° F.    |
| b. time                                         | 16 hrs.     | 16 hrs.     | 16 hrs.       | 16 hrs.     |

TABLE V

| Test Temp.           | 0.2% Y.S.<br>(KSI) | U.T.S.<br>(KSI) | El.<br>(%) | R.A.<br>(%) |
|----------------------|--------------------|-----------------|------------|-------------|
| Conventional Process |                    |                 |            |             |
| RT                   | 160                | 230             | 25         | 30          |
| 1150° F.             | 155                | 200             | 20         | 20          |
| Invention Process    |                    |                 |            |             |
| RT                   | 150                | 230             | 25         | 25          |
| 1150° F.             | 150                | 200             | 25         | 25          |

We claim:

1. Method of heat treating a nickel base superalloy article containing 40-70 volume % of the gamma-prime phase, having a gamma prime solvus temperature and a starting grain size, including the steps of:

a. producing a concentration of coarse gamma prime particles concentrated at the grain boundaries by holding the article at a first heat treat temperature about 10°-50° F. below the gamma prime solvus for at least 0.5 hour and cooling the article at about 20°-200° F./per hour to a temperature at least about 200° F. below the first heat treat temperature;

b. producing a fine dispersion of the gamma prime phase within the grains by heating to a second heat treat temperature about 10°-250° F. below the first

heat treat temperature for at least 0.5 hour and then rapidly cooling to below about 1200° F.; and

c. stabilizing the gamma prime particles within the grains by heating the article to 1200°-1500° F. for about 1-25 hours;

whereby a fatigue resistant structure containing coarse grain boundary gamma prime and fine gamma prime particles within the grains, and having a grain size essentially that of the starting grain size results.

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 82

to produce a distribution of fine (0.02-0.15 micron) gamma prime particles within the grains; and b. heating the alloy to a moderate temperature to stabilize the microstructure; whereby the alloy maintains essentially its original grain

5

size and has a microstructure comprised of original gamma prime particles and fine gamma prime particles within the grains and is resistant to fatigue crack initiation and growth.

\* \* \* \* \*

10

15

20

25

30

35

40

45

50

55

60

65